# EUROPEAN PATENT SPECIFICATION

(11) **EP 0 040 650 B1**
(45) Date of publication and mention of the grant of the patent: **28.08.1985**
(21) Application number: 80200484.6
(22) Date of filing: 22.05.1980
(51) Int. Cl.: G03G 5/10, G03G 5/02, A41H 3/02

(54) **Heat sealable electrostatic recording sheet**
Heisssiegelfähiges elektrostatisches Aufzeichnungsblatt
Feuille d'enregistrement électrostatique, collable à chaud

(43) Date of publication of application: 02.12.1981
(73) Proprietor: R.Q.O. Holding Company,Inc., Jamestown, N.Y. 14701 (US)
(72) Inventor: de Boer, Henri Gerard Jean, Delft (NL); Tellier, Jacques Carel Tristan, Rijswijk (NL); Mooyman, Johannes Marinus, Delft (NL)
(74) Representative: Kooy, Leendert Willem

## Description

### Background of the invention

This invention relates to an electrostatic recording sheet which can be heatsealed to substrate member, and more particularly to the combination of an electrically conductive base having an electric-charge-retention dielectric layer on one side and an electrically conductive heat- sealable layer on the other side.

### Brief description of the prior art

In the garment industry, heatseal paper, either diazo-sensitized or unsensitized, has come into wide spread usage. The use of heatseal whiteprinting systems in the ready-made clothing industry provides a method which both increases production and improves quality. In recent years in particular, the garment industry has been characterized by the use of faster and better machines. For the drawing and cutting rooms to keep pace with these developments, the industry has employed sensitized heatseal sheets by means of which a pattern can be placed quickly and accurately onto the material. The procedure is simple: a master marker (or original) is made by whiteprinting the patterns onto sensitized master paper. This is done by placing the pattern pieces onto a sheet of sensitized paper of the same dimensions as the material. The sensitized paper is then exposed by an electrically operated exposure unit which decomposes the sensitized layer from the spaces left uncovered by the pattern pieces. After development in a suitable developing unit, such as a GAF Pattern Printer, the master marker is ready.

From the master marker, an unlimited number of markers can be produced by the GAF Pattern Printer. In some cases, for example, for small series, variable layouts of varying material widths, the master marker can be omitted and the pattern traced directly onto translucent pattern paper. Herefrom it is possible to make several heatseal prints (copies) if desired in one operation.

The master marker is then run through the GAF Pattern Printer in contact with sensitized paper. The sensitized paper is exposed and automatically developed inside the machine and it comes out as a copy, bearing a true image of the original pattern (an exact copy of the "Master"). In the cutting room, the new copy is heatsealed onto the top layer of cloth on the cutting table. It is ironed on crosswise in order to obtain a firm bond. After the garments are cut, the paper can easily be removed from the cloth without leaving a trace.

By using this method, a library of masters is maintained and when copies are required, they can be quickly produces, thus making it totally unnecessary to store extra copies.

Heatseal materials are dimensionally stable to a very high extent and, therefore, the copy provides a dimensionally exact image of the pattern pieces. Calculated yardage remains constant and no tolerances have to be taken into account.

The garment industry, most recently, has begun to employ computerized plotters in combination with dielectric printers for producing their patterns. The dielectric paper can then be used as a master for reproduction on diazo- heatseal paper.

While it might appear to be desirable to merge the well-established heatseal print system with a dielectric printing system, such as disclosed for example in U.S. Patent 3,887,903, the dielectric coated papers are incompatible with the step of heatsealing to a fabric by using a hot iron and the required heatseal coating would provide the dielectric film with an electrically insulated surface and therefore, inoperative.

In U.S. Patent 4,139,675 heat-sealable electrostatic recording sheets have been disclosed, said sheets consisting essentially of an electrically conductive substrate sheet having a dielectric coating on a first side, said dielectric coating being composed of an electric-charge-retentive layer of a film-forming insulating or dielectric resinous polymer, said polymer also containing dispersed therein pigment particles and a heat- sealable coating on a second side, said heat- sealable coating being composed of a thermoplastic film-forming polymeric material, said thermoplastic film also containing an electrically conductive additive.

These sheets, however, are intended for applications such as making tickets, bills, receipts, outside adresses, price tags, labels, etc. i.e. applications where they are permanently stuck to a substrate and their composition is adapted to said use; they are not suitable for use in the garment industry. Thus the composition of the heat seal layer which is composed of one or more thermoplastic resins, a tackifier which is solid at room temperature and/or a plasticizer which is solid at room temperature and a conductive additive such as a quaternary ammonium salts series conductive polymer, is of such a kind that when the sheets have been heat sealed onto a layer of cloth, said sheets cannot be removed without leaving a trace; further the composition of the recording layer wherein the pigment particles besides improving the external appearance and the writing properties, also prevent blocking, nevertheless give problems with toner image smearing during the ironing process while also moving of the hot iron over the dielectric coating gives problems.

### Summary of the invention

It has now been found that a modified heat- sealable electrostatic recording sheet can be provided with a modified electric-charge-retentive layer and a modified heatseal coating to provide a dielectric paper which can both be used in electrostatic plotters and heat-sealed to a fabric by using a hot iron and without the above- mentioned problems.

In accordance with the present invention, the electric-charge-retentive layer in addition contains an anti-blocking agent, selected from the group consisting of dielectric alkaline earth metal salts of fatty acids, alkali metal salts of fatty acids, waxes, and mixtures thereof, the weight ratio of pigment to film forming resin to anti-blocking agent in said dielectric coating being either in the range from about 10/1/0.3 to 0.5/1/0.5 or in the range of from about 4/1/0.6 to 1/1/0.8.

The anti-blocking agent is preferably selected from the group consisting of dielectric alkaline earth metal salts of fatty acids, waxes, and mixtures thereof.

Indeed U.S. patent 3,709,728 mentions as a possibility to incorporate into the electrostatic recording layer of an electric recording sheet without a heat seal layer, materials such as waxes, silicones and stearate salts which have an anti-blocking action. However, these compounds are only used in very small amounts of not more than about 5% of the resin solids, which is far less than the amounts (ratios) applied according to the invention. Further only the use of ammonium stearate is examplified, said compound being used in a weight ratio of resin to stearate of 1:0.005.

Such amounts of antiblocking agent do not have a real influence on the properties of the electric-charge-retentive layer and especially on the ironing properties of such a layer in a sheet which on the other side comprises a heatseal layer. For a suitable effect on the ironing properties (smooth moving of the iron without toner image smearing, the weight ratio of pigment to film-forming resin to anti-blocking agent in the dielectric coating must be within the above- mentioned ranges.

The electric-charge-retentive layer preferably includes calcium stearate, but advantageously can include other materials having dielectric properties which are compatible with the dielectric polymeric film, as for example, waxes including the natural animal waxes, the mineral waxes and the synthetic waxes. Other alkali and alkaline earth metal salts of fatty acids can also be advantageously employed.

According to a further embodiment of the invention, the heat-sealable coating is composed of a thermoplastic film-forming polymeric material which contains an electrically conductive additive, such as a polymeric quaternary ammonium halide, and in particular, polydialkyl diallyl ammonium halide, the weight ratio in the heat seal layer of pigment to film forming resin to polymeric quaternary ammonium halide being in the range from about 1:1:0.1 to 1:6:1.

This heat seal layer does not comprise tackifiers and/or plasticizers.

Thanks to said composition these heat seal layers on cross-wise ironing give a suitable temporary bonding of the recording sheet to a layer of fabric (cloth) while removing the recording sheet does not leave a trace.

### Description of the preferred embodiments

The product of the invention is a coated paper, the paper base of which has a high degree of conductance and carrying on one side only, a substantially non-conductive or dielectric resinous layer which serves as an electric-charge-retentive layer.

The insulating resinous polymer materials forming the electric-charge-retentive layer are homopolymers or copolymers, polymerized from monomers or their derivatives, such as vinylchloride, vinylacetate, vinylidenechloride, methylacrylate, ethylacrylate, butylacrylate, 2-ethylhexylacrylate, methylmethacrylate, ethyl- methacrylate, vinylmethyl ether, vinylethylether, vinylisobutyl ether, vinylpyrrolidone, styrene, cumarone, indene, acrylonitrile, butadiene and the like, and other polymers and cellulose derivatives such as nitrocellulose, cellulose- acetate and polyamide, and mixtures of said polymers or cellulose derivatives; and particularly, the resinous polymers consist at least partially of polymeric solid particles of homopolymer or copolymer polymerized from above mentioned monomers, their derivatives or other polymers. For example, the electric-charge-retentive layer may be a film, consisting of vinylidenechloride-methylmethacrylate copolymer, which is at least partially formed by polymeric solid particles of vinylidenechloride-methylmethacrylate copolymer having a higher degree of polymerization. For another example, the electric-charge-retentive layer may be a film, consisting of isobutylacrylate-methylmethacrylate-acrylonitrile copolymer and acrylonitrile polymer, at least partially formed by polymeric solid particles of acrylonitrile polymer.

Other insulating or dielectric resins which can be used include silicone and organo-silicone resins, acid modified polyvinyl acetate, such as crotonic acid-modified polyvinyl acetate, polyvinyl butyral, wax, shellac, petroleum resins, coal tar resins, and the like. Additional binder materials disclosed in the prior are which can be used to form the dielectric coating include polyolefins, such as polyethylene and polypropylene, unmodified or oil-modified alkyd resins, styrenated alkyd resins, oil modified styrenated alkyds, saturated polyester resins, polyvinyl acetates, polyvinyl chlorides, propylene modified polyvinyl chlorides, polyvinyl butyral, vinyl chloride-vinyl acetate maleic acid terpolymers, copolymers of ethylene and vinyl acetate, acrylic acid ester polymers, methacrylic acid ester polymers, polystyrene, butadiene-styrene- copolymers, styrene-ethylene copolymers, ethyl cellulose, cellulose acetate butyrate, cellulose acetate propionate, cellulose, nitrate, sucrose esters (e.g. sucrose benzoate and the like) and polysulfones.

The dielectric coating can include pigments such as calciumcarbonate, zincsulphide, lithopone, magnesiumoxide, ammoniumstearate, bariumsulfate, organophilic pigment (containing ethylene/acrylic acid copolymer) and clay.

The electric-charge-retentive layer requires the use of an anti-blocking or lubrication agent in order to facilitate a smooth moving of the iron when the heatsealable layer is being fused to a fabric.

While calcium stearate is the preferred agent, other agents can be used, as for example, alkali and alkaline earth metal salts of fatty acids and waxes, including the natural animal waxes, such as beeswax, spermaceti, lanolin and shellac wax; the vegetable waxes, such as carnauba, candelilla, bayberry and sugarcane; and mineral waxes, such as the fossil or earth waxes and petroleum waxes, such as paraffin and microcrystalline petrolatum. The synthetic waxes incude ethylene polymers and polyol ether- esters, such as sorbitol, chlorinated naphthalenes and hydrocarbon waxes. The wax must have good dielectric properties and be compatible with the binder and pigment.

Beside improved ironing properties of the coating, and prevention of toner image smearing during the ironing process, the anti-blocking or lubricating agent has been found to provide improved liquid toner adhesion.

The unique combination of a dielectric- conductive heat-sealable sheet was found to have a surprising cost savings. Cheap, relatively low conductive base materials were found to produce the same results heretofore attainable only with more expensive, higher conductivity base materials. The improved results appear to be, at least in part, attributable to the penetration of the conductive heatseal coating.

The heatseal coating is provided with a material which renders the coating electrically conductive, but does not adversely affect the heatseal properties of the coating. Because of the nature of electrically conductive materials, the following problems can be encountered when modifying a heatseal material:
1. loss of heatseal properties; and
2. transfer of part of heatseal coating to the underlying fabric.

Therefore the selection of a conductive material is critical and it has been found that the following classes of materials produce the desired results:
I. polymeric quaternary ammonium halides
IA. poly(diallyl-dialkyl ammonium halides
IB. polydialkyl-divinyl ammonium halides
II. ammonium salts of alkylarylsulfonates
III. electrolytes or conductive salts
IIIA. calcium, sodium or lithium chloride, sodium or ammonium nitrate
IV. carbon black
V. metal powders
VI. surface active agents

The heatsealable filmformers which can be used include polyvinylacetate, copolymer of vinylchloride and vinylacetate, copolymer or vinylacetate and ethylene, copolymer of vinylchloride and maleicacid ester and aqueous dispersion of these.

The heatseal layer can include pigments such as calciumcarbonate, zincsulphide, china clay, titaniumdioxide, oxidized starch and kaolin.

The function of the pigment, preferably calciumcarbonate, in the heatseal layer, is to reduce the tack of the conductive resin component of the coating and thus to prevent blocking of the material on the roll.

The base material, that is, the conductive layer, typically has a surface resistivity in the range of from 4.10⁶ to 7.10⁶ 0/square and a bulk resistivity of about 3.10⁵ Ω cm. However, in the combination of the instant invention, cheaper materials can be employed, having a surface resistivity in the range from about 6.10' to 8.10' 0/square and a bulk resistivity on the order of 4.10⁶ 0 cm.

The process of computerized grading of pattern pieces, interactive marker making, and the drawing of full scale apparel marker in preparation for cloth cutting, is disclosed in U.S patent 3,887,903.

A programmed voltage is applied to an array of densely spaced writing nibs embedded in a stationary writing head. Upon digital command, the nibs selectively create minute electrostatic dots on a dielectric paper as it passes over the writing head. The paper is then exposed to liquid toner to produce a visible permanent image. The paper is then heatsealed to any substrate, such as a woven fabric by applying heat and pressure by means of conventional iron.

The electrostatic recording sheet can be prepared in accordance with the known coating techniques.

### Example 1

The dielectric coating is prepared by forming a dispersion in 80 I of toluene, of 37.5 kg of an acrylicmethacrylic copolymer, sold under the Trademark E-322 by DeSoto, Inc. (DesPlaines, Illinois), 32.5 kg calcium carbonate, 5 kg calcium stearate and 90 g of an optical brightener sold under the Trademark Uvitex OB, by Ciba-Geigy, and applying the coating to a conductive base material. The conductive base is a material sold under the Trademark DEC-Base No. 358 by Schoeller. The coating weight on a dry basis is 9 grams per square meter (g/m²).

The heatseal coating is prepared by forming, in 70 I of methanol, a dispersion of 18.7 I of ethylacetate and 25 kg of a polyvinylacetate sold under the Trademark Vinnapas B60, by Wacker, 10 kg of polydiallyldimethyl ammonium chloride, sold under the Trademark Chemviron 261 by Merck, and 10 kg of calcium carbonate. The Chemviron 260 contains 40% solids by weight. The coating weight on a dry basis is 20 g/_{M}².

### Example II

In accordance with the procedures outlined in U.S. Patent 3,709,728, the disclosure of which is herein incorporated by reference, an electrostatic recording sheet is produced having a 5.8 g/m² coating comprising a first layer of 100 parts SBR latex, 2.5 parts melamine formaldehyde and 50 parts pigment (barium sulphate and zinc sulphide) and a second layer of (2.2 g/m²) of 100 parts carboxylated polyvinyl acetate, 0.5 parts ammonium stearate and 50 parts pigment (barium sulphate and zinc sulphate).

The first coating is applied to the substrate by mixing with water to produce a solids content of approximately 50%. The coating is cured and rendered resistant to water by subjecting it to 5 minutes of heating at 82°C.

The second coating composition is similarly mixed with sufficient water to yield a 50% solids content and then adjusted to a pH of approximately 9 by the addition of ammonium hydroxide. Curing is achieved by heating at 71°C for 5 minutes, driving off the ammonia and rendering the coating insoluble in water.

As the next treatment, the coated paper was coated over its back face with an aqueous solution of sodium nitrate, at 25% concentration. Such was applied by spraying it onto the paper web, at a rate of about 4.4 g/m² (solids basis).

When measured for surface resistivity, the front side of the copy sheet exhibits a surface resistivity of 10⁷ ohms per square, and the back side of the copy sheet exhibits a surface resistivity of 10³ ohms per square.

A heatseal coating is then applied to the back side in accordance with the procedures of Example I.

The recording blank can then be processed to print thereon alphanumeric information, using electrographic short pulse printing procedures.

There are various forms of equipment for electrographic pulse printing available commercially, exemplified by the Printipix Tube produced by Scientific Recorders, the Clevite 4800 made by Gould, the Info-Max and the computer oriented electrostatic printer of Versatec, Inc. Such a printer may include a bank of styli or electrodes which form the printing head in the machine. The recording blank is moved across this printing head, while supported on a backup support means which comprises a backup electrode to produce charged regions on the sheet. DC voltage pulses are applied between selected ones of the electrodes and the backup support forming on opposing electrode. The voltage applied between opposed electrodes ordinarily ranges between a threshold voltage of about 340 volts and 1100 volts.

Demonstrating the utility of the recording blank of the invention can be printed in an electrographic pulse printing machine using pulses of 100 microsecond duration. Charged regions on the recording blank are developed using conventional developer material to produce a visible image. Excellent prints exhibiting good image density and resolution are produced by this system.

### Example III

In accordance with the procedures of British Patent 1,332,139 the disclosure of which is herein incorporated by reference, a heatsealableelectro- static recording sheet can be produced using as the dielectric layer, a film produced from a dispersion of 100 parts SBR latex; 10 parts 30% butadiene, 55% methylmethacrylate, 15% methacrylic acid; and 2 parts polyoxyethylene lauryl- ether. Additionally 10 parts of calcium stearate is employed in the dispersion.

Except with respect to the foregoing, the procedures of Example I are followed to produce a heatsealable electrostatic coating.

### Example IV

The procedures of Example I are followed, except a 5 11m thickness of a copolymer of vinylidene chloride and methylmethacrylate are used as the dielectric film former, in accordance with the procedures disclosed in U.S. Patent 3,634,135, the disclosure of which is incorporated herein by reference.

### Example V

The procedures of Example IV are followed except that the dielectric film is formed from 55 parts vinylidene chloride, 40 parts methylmethacrylate and 5 parts acrylic acid in accordance with the teachings of U.S. Patent 3,634,135.

### Example VI

The procedure of Example I is followed, except that the dielectric film is applied as a coating of 8 g/m² of 935 g polyvinyl acetate, 498 g clay, 125 g barium sulfate with 5,000 cm³ water containing 200 cm³ of 28% NH₄0H as disclosed in U.S. Patent 3,264,137, the disclosure of which is incorporated herein by reference. Additionally,100 g of calcium stearate is employed in the coating.

### Example VII

The procedure of Example I is followed, except that in accordance with the disclosure of U.S. patent 3,639,640, the disclosure of which is herein incorporated by reference, the conductive substrate is formed by coating and impregnation on a paper having a basis weight of 76 g/m² with a solution of 12 parts of a vinylbenzyltrimethyl ammonium chloride polymer having a 32% solids content and sold by the Dow Chemical Company under the designation "DOW QX 2611.7", 30 parts of methanol and 67.5 parts of ethanol to provide, after drying an electrically conductive coating on one side thereof of 1.56 g/m² (4%) and 0.39 g/m² (1 %) on the other side thereof. The side having the 4% coating on conductive resin is then coated with a dispersion of 10 parts of a polyvinyl butyral resin (sold by Union Carbide Corporation under the designation "Bakelite XYHL"), 11.6 parts of lithophone, 29.6 parts of ethanol and 48.8 parts of toluene to provide, after drying, a thickness ot from about 1.25 to 6.25 µm. Additionally, 2 parts of calcium stearate is incorporated in the dispersion. The heatseal coating is then applied to the 1% coating.

### Example VIII

In accordance with the disclosure of U.S. Patent 3,652,268, the disclosures of which are incorporated herein by reference, a conductive substrate can be formed as described in Examples I, II and III of the patent. The dielectric layer can be formed as described in Examples IV and V of the patent, except that 10% by weight calcium stearate is incorporated in the dielectric coating composition. The heatseal coating is then formed as described in Example I.

### Example IX

An electrostatic recording sheet can be formed following the procedure of Example I or II of U.S. Patent 3,216,853, the disclosure of which is herein incorporated by reference, except that in Example I, 150 parts by weight of calcium stearate is incorporated and in Example II 5 parts of weight of calcium stearate is incorporated with the polyvinyl acetate coating.

The conductive side of the paper is then coated with the heatseal coating as set forth in Example I.

### Example X

An electrostatic recording sheet is prepared by coating a paper sheet with titanium dioxide and polyvinyl benzyltrimethyl ammonium chloride as described in the Examples of U.S. patent 3,759,744, the disclosure of which is herein incorporated by reference. The dielectric coating employs 2.5 parts carboxylated polyvinyl acetate, 1 part CaC0₃ and 0,2 part calcium stearate.

The heatseal coating is prepared as disclosed in Example I.

### Example XI

The procedures of previous examples can be followed in combination with a heatseal layer produced from an aqueous, conductive formulation as follows:

A coating weight, on a dry basis of 20 g/m² can be produced. Propiofan 590 is a trademark of the BASF Company for a vinyl propionate-acrylate copolymer dispersion used to produce flexible films.

Vinamul 6705 is a trademark of the Scado Company, Zwolle, Netherlands, for a vinyl acetate-ethylene copolymer.

In the heatseal layer, the ratio of pigment to film-forming resin to conductive additive can be in the range from 1/1/0.1 to 1/6/1. However, the range from 1/2/0.3 to 1/4/0.7 is preferred because this range gives both adequate heatseal properties and adequate conductivity level.

## Claims

1. A heat-sealable electrostatic recording sheet consisting essentially of an electrically conductive substrate sheet having a dielectric coating on a first side, said dielectric coating being composed of an electric-charge-retentive layer of a film-forming insulating or dielectric resinous polymer, said polymer also containing dispersed therein pigment particles and a heat-sealable coating on a second side, said heat-sealable coating being composed of a thermoplastic film-forming polymeric material, said thermoplastic film also containing an electrically conductive additive, characterized in that the electric-charge-retentive layer in addition contains an anti-blocking agent, selected from the group consisting of dielectric alkaline earth metal salts of fatty acids, alkali metal salts of fatty acids, waxes, and mixtures thereof, the weight ratio of pigment to film-forming resin to anti-blocking agent in said dielectric coating being either in the range from about 10/1/0.3 to 0.5/1/0.5, or in the range from about 4/1/0.6 to 1/1/0.8.

2. The heat-sealable electrostatic recording sheet of claim 1, characterized in that the heat seal layer comprises a film forming polymeric material, pigment and polymeric quaternary ammonium halide, the weight ratio in the heat seal layer of pigment to film forming resin to polymeric quaternary ammonium halide being in the range from about 1/1/0.1 to 1/6/1.

3. The heat-sealable electrostatic recording sheet of claim 1 or 2, wherein the weight ratio in the heat seal layer of the pigment to film-forming resin to conductive additive is in the range from about 1/2/0.3 to 1/4/0.7.

4. The heatsealable electrostatic recording sheet mentioned in one of the preceding claims, wherein the electrically conductive additive is polydimethyl diallyl ammonium chloride.

## Patentansprüche

1. Heißsiegelfähiges, elektrostatisches Aufzeichnungsblatt, das im wesentlichen aus einem Blatt aus elektrisch leitendem Substrat mit einer dielektrischen Beschichtung auf einer Seite, welche dielektrische Beschichtung aus einer die elektrische Ladung haltenden Schicht aus einem filmbildenden, isolierenden oder dielektrischen, harzartigen Polymer besteht, das auch darin dispergierte Pigmentteilchen enthält, und einer heißsiegelfähigen Beschichtung auf der zweiten Seite besteht, welche heißsiegelfähige Beschichtung aus einem thermoplastischen, filmbildenden Polymermaterial besteht, wobei der thermoplastische Film auch einen elektrisch leitenden Zusatz enthält, dadurch gekennzeichnet, daß die die elektrische Ladung haltende Schicht zusätzlich ein Antiblockmittel enthält, das aus der Gruppe ausgewählt ist, die aus dielektrischen Erdalkalimetallsalzen von Fettsäuren, Alkalimetallsalzen von Fettsäuren, Wachsen und Mischungen davon besteht, wobei das Gewichtsverhältnis von Pigment zum filmbildenden Harz zum Antiblockmittel in der dielektrischen Beschichtung entweder im Bereich von etwa 10/1/0,3 bis 0,5/1/ 0,5 oder im Bereich von etwa 4/1/0,6 bis 1/1/0,8 ist.

2. Heißsiegelfähiges, elektrostatisches Aufzeichnungsblatt nach Anspruch 1, dadurch gekennzeichnet, daß die Heißsiegelschicht ein filmbildendes Polymermaterial, Pigment und polymeres, quaternäres Ammoniumhalogenid umfaßt, wobei das Gewichtsverhältnis in der Heißsiegelschicht von Pigment zu filmbildendem Harz zu polymerem, quaternärem Ammoniumhalogenid im Bereich von etwa 1/1/0,1 bis 1/6/1 ist.

3. Heißsiegelfähiges, elektrostatisches Aufzeichnungsblatt gemäß Anspruch 1 oder 2, dadurch gekennzeichnet, daß das Gewichtsverhältnis in der Hießsiegelschicht von Pigment zum filmbildenden Harz zu leitendem Zusatz im Bereich von etwa 1/2/0,3 bis 1/4/0,7 ist.

4. Heißsiegelfähiges, elektrostatisches Aufzeichnungsblatt nach einem der vorhergehenden Ansprüche, dadurch gekennzeichnet, daß der elektrisch leitende Zusatz Polydimethyldiallylammoniumchlorid ist.

## Revendications

1. Feuille d'enregistrement électrostatique collable à chaud, consistant essentiellement en une feuille de substrat conducteur d'électricité ayant un enduit dielectrique sur une première face, ledit enduit diélectrique étant composé d'une couche de rétention de charges électriques d'un polymère résineux filmogène isolant ou diélectrique, ledit polymère contenant également en dispersion des particules de pigment et un enduit collable par la chaleur sur une seconde face, ledit enduit collable par la chaleur étant composé d'une matière polymère thermoplastique filmogène, ladite pellicule thermoplastique contenant également un additif conducteur d'électricité, caractérisée en ce que la couche de rétention des charges électriques contient en outre un agent d'antiblocage choisi dans le groupe comprenant les sels diélectriques de métaux alcalino-terreux d'acides gras, les sels de métaux alcalins d'acides gras, les cires, et leurs mélanges, le rapport pondéral du pigment à la résine filmogène à l'agent d'antiblocage dans ledit enduit diélectrique étant soit dans l'intervalle d'environ 10/1/0,3 à 0,5/1/0,5 soit dans l'intervalle d'environ 4/1/0,6 à 1/1/0,8.

2. Feuille d'enregistrement électrostatique collable à chaud selon la revendication 1, caractérisée en ce que la couche collable à chaud comprend une matière polymère filmogène, un pigment et un halogénure polymère d'ammonium quaternaire, le rapport pondéral dans la couche collable à chaud du pigment à la résine filmogène à l'halogénure polymère d'ammonium quaternaire étant d'environ 1/1/0,1 à 1/6/1.

3. Feuille d'enregistrement électrostatique collable à chaud selon la revendication 1 ou 2, dans laquelle le rapport pondéral dans la couche collable à chaud du pigment à la résine filmogène à l'additif conducteur est d'environ 1/2/0,3 à 1/4/0,7.

4. Feuille d'enregistrement électrostatique collable à chaud selon l'une des revendications précédentes, dans laquelle l'additif conducteur d'électricité est le chlorure de polydiméthyl- diallyl-ammonium.
